

# United States Patent [19]

Isailingold et al.

[11] 3,862,256

[45] Jan. 21, 1975

[54] **METHOD FOR PREPARING MONO- AND DI-OLEFINE HYDROCARBONS**

[76] Inventors: **Anatoly Lvovich Isailingold**, ulitsa Chekhova, 25, kv. 31; **Veniamin Anatolievich Levin**, Svobody, 75/37, kv. 24; **Fedor Semenovich Pilipenko**, zhskaya naberezhnaya, 25/2, kv. 7; **Tatyana Pavlovna Vernova**, Uglichskoe shosse, 10, kv. 40; **Gennady Arkadievich Stepanov**, ulitsa Pervomaiskaya, 9, kv. 3; **Alexandr Nikitich Bushin**, ulitsa Pervomaiskaya, 9, kv. 21; **Boris Vasilievich Sirotkin**, ulitsa 1 Zhilaya, 6, kv. 23; **Valentin Vasilievich Kozin**, ulitsa Kolesovoi, 34, kv. 18; **Mark Ekhetskelevich Basner**, prospekt Lenina, 36, kv. 30; **Aida Vladimirovna Erofeeva**, prospekt Lenina, 11/74, kv. 30; **Nina Prokopievna Peshkova**, Leningradsky prospekt, 59, kv. 49; **Luiza Saidovna Tuktarova**, ulitsa Junosti, 5, kv. 15; **Yakov Yakovlevich Kirnos**, ulitsa Pervomaiskaya, 9, kv. 5; **Ruslan Konstantinovich Mikhailov**, ulitsa Tolbukhina, 45/14, kv. 43; **Nikolai Zakharovich Dolinin**, prospekt Lenina, 23, kv. 26; **Jury Nikolaevich Rastvorov**, Tutaevskoe shosse, 51, kv. 50; **Valeria Lvovna Eratova**, ulitsa Bljukhera, 36, kv. 5, all of Yaroslavl, U.S.S.R.

[22] Filed: Aug. 7, 1972

[21] Appl. No.: 278,654

[52] U.S. Cl. .... 260/680 E, 252/468, 260/683.3

[51] Int. Cl. .... C07c 5/18

[58] Field of Search ..... 260/680 E, 683.3

[56] **References Cited**

UNITED STATES PATENTS

|           |         |                      |           |
|-----------|---------|----------------------|-----------|
| 3,119,111 | 1/1964  | McDonald et al. .... | 260/680 E |
| 3,308,191 | 3/1967  | Bajars .....         | 260/683.3 |
| 3,308,196 | 3/1967  | Bajars .....         | 260/680 D |
| 3,308,200 | 3/1967  | Bajars .....         | 260/680 D |
| 3,356,757 | 12/1967 | Roth et al. ....     | 260/683.3 |
| 3,678,124 | 7/1972  | Stepanov et al. .... | 260/680 E |
| 3,718,707 | 2/1973  | Knippa et al. ....   | 260/678   |

Primary Examiner—Paul M. Coughlan, Jr.

[57] **ABSTRACT**

A method for the production of mono- and diolefinic hydrocarbons by subjecting paraffinic hydrocarbons to catalytic oxidative dehydrogenation at 400° to 700° in the presence of a catalyst comprising oxygen-containing compounds of molybdenum and magnesium taken in a molybdenum/magnesium atomic ratio of 1:0.9 to 1:357, optional components of said catalyst being oxygen-containing compounds of cobalt, iron, chromium, vanadium, nickel, silicon, antimony, boron, gadolinium, dysprosium, gallium, bismuth, titanium, zirconium or niobium.

19 Claims, No Drawings

## METHOD FOR PREPARING MONO- AND DI-OLEFINE HYDROCARBONS

The invention relates to the for preparing mono- and di-olefinic hydrocarbons.

Said hydrocarbons are used in the synthesis of various organic compounds, and in the manufacture of synthetic rubbers in particular.

Methods are known in the art for preparing mono- and di-olefinic hydrocarbons by catalytic oxidative dehydrogenation of paraffin hydrocarbons.

Thus, for example, a method is known for preparing *n*-butenes and butadiene by the oxidative dehydrogenation of *n*-butane on the phosphomolybdate of sodium or lithium at 400° – 650°C. The yield of butadiene in reactors with a fluidized catalyst is 17.2 percent, the conversion of *n*-butane being 28 percent. The selectivity with the stationary catalyst bed does not exceed 41 percent, the conversion of *n*-butane being 42 percent (of U.S. Pat. No. 3,119,111).

A method is also known for oxidative dehydrogenation of paraffin hydrocarbons on an oxidic aluminophosphate catalyst at a temperature of 420° – 660°C. According to this method, the conversion of *n*-butane does not exceed 40 percent, the total selectivity with respect to butadiene and *n*-butenes being 39 – 42 percent, and the ratio  $C_4H_6 : C_4H_8$  in the reaction products being 0.16 – 0.46 (cf. U.S. Pat. No. 3,320,331).

Also known is a method for preparing mono- and di-olefinic hydrocarbons by the oxidative dehydrogenation of paraffin hydrocarbons at a temperature from 400° to 700°C and molar ratio of oxygen to the paraffin hydrocarbon of 0.1 – 3, in the presence of an inert diluent, e.g. water vapor, nitrogen, argon, helium or their mixtures, on a catalyst, which is an oxy compound of molybdenum and/or tungsten, and of at least one of the following metals: chromium, manganese, iron, nickel or cadmium. During oxidative dehydrogenation of *n*-butane according to this method, the conversion of *n*-butane is 55.5 percent, the total selectivity with respect to butadiene and *n*-butenes being 43.2 percent. The yield of butadiene is 19.1 percent (cf. British Pat. No. 1,197,537).

The disadvantages inherent in these methods are low conversion of the hydrocarbon stock material and low selectivity with respect to the main products.

The object of this invention is to work out a method for catalytic oxidative dehydrogenation of paraffin hydrocarbons into mono- and di-olefinic hydrocarbons which would ensure higher conversion of the starting material and higher yields of the main products.

In accordance with this and other objects the invention consists in oxidative dehydrogenation of paraffin hydrocarbons at a temperature from 400° to 700°C and the molar ratio of oxygen to the paraffin hydrocarbon of 0.1 – 3, in the presence of an inert diluent, such as water vapor, nitrogen, argon, helium or mixtures thereof, on a catalyst containing oxy compounds of molybdenum. The catalyst according to the invention contains also oxy compounds of magnesium and absorbs in the infra-red region of the spectrum, the wave numbers being 780  $\text{cm}^{-1}$ , 830  $\text{cm}^{-1}$ , 890  $\text{cm}^{-1}$ , 950  $\text{cm}^{-1}$  and 970  $\text{cm}^{-1}$ .

It is recommended that use should be made of a catalyst in which the atomic ratio of Mo to Mg is from 1 : 0.9 to 1 : 357, preferably from 1:3.6 to 1:68.5.

With the purpose of increasing the yield of the main products, it is recommended to use a catalyst which in addition to the above compounds also contains oxy compounds of at least one of the following elements: 5 cobalt, iron, chromium, vanadium, silicon or nickel. The content of the oxy compounds of at least one of the above metals in the catalyst can be varied from 0.01 to 20 percent by weight calculated with reference to the metal oxides.

- 10 In order to increase the yield of the main products, it is possible also to use a catalyst which, in addition to the oxygen-containing compounds of molybdenum and magnesium, also contains oxy compounds of at least one of the following metals: antimony, boron, gadolinium, dysprosium, gallium, bismuth, titanium, zirconium or niobium. The amount of the oxy compounds of at least one of the above metals in the catalyst can vary from 0.01 to 5 percent by weight calculated with respect to the metal oxides.
- 20 In addition to the above two cases, the yield of the main products can also be increased by using a catalyst which in addition to the oxy compounds of molybdenum and magnesium, also contains oxy compounds of at least one of the following elements: cobalt, iron, 25 chromium, vanadium, silicon or nickel, and also oxy compounds of at least one of the following metals: antimony, boron, gadolinium, dysprosium, gallium, bismuth, titanium, zirconium or niobium. The amount of the oxy compounds of the above metals in the catalyst can vary within the above specified limits (from 0.01 to 20 percent by weight and from 0.01 to 5 percent by weight respectively).

In order to increase the mechanical strength of the catalyst so that the process can be carried out with a fluidized catalyst, the latter should be applied onto carriers, such as aluminosilicates, silica gel or alumina.

In the proposed method according to the invention, the oxidative dehydrogenation of paraffin hydrocarbons was effected at temperatures within a wide range (from 400° to 700°C), the molar ratio of oxygen to the paraffin hydrocarbon of 0.1 – 3 and the rate of the starting hydrocarbon input of 20 to 1,000 hour<sup>-1</sup>. The oxidative dehydrogenation of the hydrocarbons was carried out in the presence of an inert diluent, e.g. water vapor, nitrogen, argon, helium, or mixtures thereof. The preferable molar ratio of the inert diluent to the paraffin hydrocarbon should be 1 : 1 to 40 : 1. Carrying out the process in the presence of inert diluents improves the conditions for removal of heat and increases the selectivity of the process.

Most preferable are the following conditions for the process: temperature from 500° to 650°C, the molar ratio of oxygen to the paraffin hydrocarbon of 0.5 – 2, and input rate of the starting hydrocarbons, 20– 200 hour<sup>-1</sup>.

The catalyst to be used according to the invention can be prepared by any of the known methods, for example, by precipitation, impregnation, etc. The proportions of the active components in the catalyst can vary within wide limits.

Mono-olefinic hydrocarbons (for example, *n*-butenes, isoamylenes) produced in the process, can be returned into the reaction zone so that the corresponding di-olefinic hydrocarbons can be produced under the given conditions of the process.

Owing to the use in the method according to the invention of the above described catalyst, the process of

oxidative dehydrogenation of paraffin hydrocarbons into mono- and di-olefinic hydrocarbons is carried out with a high conversion of the starting hydrocarbon raw material (to 70 percent) and high yields of the main products (to 45 mol percent).

For a better understanding of the present invention, it will be illustrated by examples of its practical embodiment. (The quantities of oxy compounds of cobalt, iron, chromium, vanadium, silicon, nickel, antimony, boron, gadolinium, dysprosium, gallium, bismuth, titanium, zirconium and niobium are given with reference to the oxides of the respective elements).

#### EXAMPLE 1

Oxidative dehydration of *n*-butane was carried out in a reactor with a stationary bed and a catalyst consisting of oxy compounds of magnesium, molybdenum and vanadium. The catalyst was prepared by the following procedure. 45 g of magensia were mixed with a solution of 6.15 g of ammonium paramolybdate in distilled water. The moist paste was shaped into granules, dried at 110° - 120°C for 10 hours and calcined at 700°C for 10 hours. The calcined granules were then impregnated with a solution of 0.44 g of ammonium metavanadate in 12.5 ml of distilled water and dried at 110° - 120°C for 10 hours. The finished catalyst contained molybdenum, magnesium (Mo to Mg atomic ratio being 1 : 31.4) and 3 percent by weight of vanadium pentoxide  $V_2O_5$ . The catalyst absorbed in the infra-red region of the spectrum, the wave numbers being 780  $\text{cm}^{-1}$ , 830  $\text{cm}^{-1}$ , 890  $\text{cm}^{-1}$ , 950  $\text{cm}^{-1}$  and 970  $\text{cm}^{-1}$ .

The infra-red absorption spectrum of the catalyst was obtained by suspending its sample in vaseline oil. The record was made on model UR-10 spectrophotometer (K. Zeiss, Jena).

The process of oxidative dehydrogenation of *n*-butane with the said catalyst was carried out at a temperature of 570°C, the molar ratio of *n*-butane to oxygen and to water vapor was 1 : 1.5 : 20, and the input rate of the *n*-butane was 50 hour<sup>-1</sup>. The charge of the catalyst was 10 cu.cm.

The yield of butadiene with respect to the *n*-butane passed through was 36.6 mol percent and of *n*-butenes, 6.4 mol percent, the selectivity being 54.7 and 9.6 mol percent respectively. The conversion of *n*-butane was 67.0 percent.

#### EXAMPLE 2

The oxidative dehydrogenation of *n*-butane was carried out in a reactor with a suspended bed of a catalyst consisting of oxy compounds of magnesium, molybdenum and vanadium. The catalyst was prepared by the method as described in Example 1 and contained molybdenum & magnesium atoms in the ratio of 1 : 32.1, and also 1 percent by weight of  $V_2O_5$ . The catalyst had an absorption spectrum similar to that specified in Example 1.

The oxidative dehydrogenation of *n*-butane was carried out at a temperature of 620°C, the molar ratio of *n*-butane to oxygen and to water vapor was 1 : 1.5 : 20 and the volumetric input rate for *n*-butane was .50 hour<sup>-1</sup>. The charge of the catalyst was 100 cu.cm.

The yield of butadiene with respect to the *n*-butane passed through was 34.2 mol percent, and of butenes, 3.8 mol percent, the selectivity being 48.8 and 5.6 mol percent respectively. The conversion of *n*-butane was 70.5 percent.

#### EXAMPLE 3

The oxidative dehydrogenation of *n*-butane was carried out in a reactor with a stationary bed of the catalyst as described in Example 1. The process temperature was 450°C, the molar ratio of *n*-butane to oxygen and to water vapor was 1 : 1.5 : 10 and the volumetric input rate of *n*-butane was 20 hour<sup>-1</sup>. The charge of the catalyst was 10 cu.cm.

10 The yield of butadiene with respect to the *n*-butane passed through was 11.6 mol percent, and of *n*-butenes, 3.3 mol percent, the selectivity being 38.7 and 11.0 mol percent respectively. The conversion of *n*-butane was 30.0 percent.

#### EXAMPLE 4

The oxidative dehydrogenation of *n*-butane was carried out in a reactor with a stationary bed of a catalyst containing oxy compounds of magnesium, molybdenum and chromium. The catalyst was prepared by the method described in example 1, and contained molybdenum and magnesium atoms in the ratio of 1.32.3 and also 0.5 percent by weight of  $\text{Cr}_2\text{O}_3$ . The catalyst had an absorption spectrum in the infra-red region similar to that specified in Example 1.

20 The oxidative dehydrogenation of *n*-butane was carried out at a temperature of 630°C, the molar ratio of *n*-butane to oxygen and to water vapor 1 : 1.5 : 20, and the volumetric input rate of *n*-butane was 50 hour<sup>-1</sup>. The charge of the catalyst was 10 cu.cm.

25 The yield of butadiene with respect to the *n*-butane passed through was 26.6 mol percent, and of *n*-butenes, 4.0 mol percent, the selectivity being 45.7 and 6.8 mol percent respectively. The conversion of *n*-butane was 58.2 percent.

#### EXAMPLE 5

The oxidative dehydrogenation of *n*-butane was carried out in a reactor with a stationary bed of a catalyst consisting of oxy compounds of magnesium, molybdenum and cobalt. The catalyst was prepared by the method described in Example 1, and contained molybdenum and magnesium atoms in a ratio of 1 : 32.4, and also 0.1 percent by weight of  $\text{Co}_3\text{O}_4$ . The catalyst had an IR spectrum similar to that described in Example 1.

30 The process temperature was 630°C, the molar ratio of *n*-butane to oxygen and to water vapor was 1 : 1.5 : 20, and the volumetric input rate of *n*-butane was 50 hour<sup>-1</sup>. The charge of the catalyst was 10 cu.cm.

35 The yield of butadiene with respect to the *n*-butane passed through was 22.6 mol percent, and of *n*-butenes, 3.6 mol percent, the selectivity being 45.8 and 7.3 mol percent respectively. The conversion of *n*-butane was 39.4 percent.

#### EXAMPLE 6

The oxidative dehydrogenation of *n*-butane was carried out in a reactor with a stationary bed of a catalyst consisting of oxy compounds of magnesium, molybdenum and iron. The catalyst was prepared by the method described in Example 1, and contained molybdenum and magnesium atoms in the ratio of 1 : 32.4, and also 0.1 percent by weight of  $\text{Fe}_2\text{O}_3$ . The IR absorption spectrum of the catalyst was the same as in Example 1.

40 The process temperature was 630°C, the molar ratio of *n*-butane to oxygen and to water vapor was 1 : 1.5

: 10 and the rate of delivery of n-butane was 50 hour<sup>-1</sup>. The input charge of the catalyst was 10 cu.cm.

The yield of butadiene with respect to the n-butane passed through was 33.5 mol percent and of n-butenes, 8.9 mol percent, the selectivity being 41.3 and 10.9 mol percent respectively. The conversion of n-butane was 81.1 percent.

#### EXAMPLE 7

The oxidation dehydrogenation of n-butane was carried out in a reactor with a stationary bed of a catalyst consisting of oxy compounds of magnesium, molybdenum and silicon. The catalyst was prepared by the method described in Example 1, and contained molybdenum and magnesium atoms in the ratio of 1 : 31.7, and also 2 percent by weight of SiO<sub>2</sub>. The IR absorption spectrum of the catalyst was similar to that in Example 1.

The process was carried out at a temperature of 630°C, the molar ratio of n-butane to oxygen and to water vapor was 1 : 1.5 : 20, the input of n-butane was 25 hour<sup>-1</sup>. The charge of the catalyst was 10 cu.cm.

The yield of butadiene with respect to the n-butane passed through was 30.3 mol percent, and of n-butenes, 6.1 mol percent, the selectivity being 47.3 and 9.4 mol percent respectively. The conversion of n-butane was 64.2 percent.

#### EXAMPLE 8

The oxidative dehydrogenation of n-butane was carried out in a reactor with a stationary bed of a catalyst consisting of oxy compounds of magnesium, molybdenum, silicon and vanadium. The catalyst was prepared by the method described in Example 1, and contained molybdenum and magnesium atoms in the ratio of 1 : 30.2, and also 1 percent by weight of V<sub>2</sub>O<sub>5</sub> and 5 percent by weight of SiO<sub>2</sub>. The catalyst had an absorption spectrum in the IR region similar to that in Example 1.

The process was carried out at a temperature of 605°C, the molar ratio of n-butane to oxygen and to water vapor was 1 : 1.5 : 20, and the rate of n-butane was 100 hour<sup>-1</sup>. The charge of the catalyst was 12.5 cu.cm.

The yield of butadiene with respect to the n-butane passed through was 33 mol percent, and of n-butenes, 5.5 mol percent, the selectivity being 51.8 and 8.7 mol percent respectively. The conversion of n-butane was 63.6 percent.

#### EXAMPLE 9

The oxidative dehydrogenation of n-butane was carried out in a reactor with a stationary bed of a catalyst consisting of oxy compounds of magnesium, molybdenum, iron and vanadium. The catalyst was prepared by the method described in Example 1, and contained molybdenum and magnesium atoms in the ratio of 1 : 31.7, and also 1 percent by weight of Fe<sub>2</sub>O<sub>3</sub> and 1 percent by weight of V<sub>2</sub>O<sub>5</sub>. The IR absorption spectrum of the catalyst was as in Example 1.

The process temperature was 615°C, the molar ratio of n-butane to oxygen and to water vapor was 1 : 1.5 : 20, and the volumetric input rate of n-butane was 50 hour<sup>-1</sup>. The charge of the catalyst was 10 cu.cm.

The yield of butadiene with respect to the n-butane passed through was 38.3 mol percent, and of n-butenes, 3.7 mol percent, the selectivity being 54.6 and 5.4 mol

percent respectively. The conversion of n-butane was 70.0 percent.

#### EXAMPLE 10

The oxidative dehydrogenation of isopentane was carried out in a reactor with a stationary bed of a catalyst similar to that used in Example 2.

The process was carried out at a temperature of 605°C, the molar ratio of isopentane to oxygen and to water vapor was 1 : 2.5 : 20, and the input rate of isopentane was 125 hour<sup>-1</sup>. The charge of the catalyst was 10 cu.cm.

The yield of isoprene with respect to the passed isopentane was 15.4 mol percent, and of isoamylenes, 2.6 mol percent, the selectivity being 40 and 7 mol percent respectively. The conversion of isopentane was 38.5 percent.

#### EXAMPLE 11

The oxidative dehydrogenation of isopentane was carried out in a reactor with a stationary bed of a catalyst similar to that used in Example 9.

The process was carried out at a temperature of 617°C, the molar ratio of isopentane to oxygen and to water vapor was 1 : 1.5 : 20, and the input rate of isopentane was 50 hour<sup>-1</sup>. The charge of the catalyst was 10 cu.cm.

The yield of isoprene with respect to the isopentane passed through was 15.5 mol percent, and of isoamylenes, 5.5 mol percent, the selectivity being 35.3 and 12.5 mol percent respectively. The conversion of isopentane was 44 percent.

#### EXAMPLE 12

The oxidation dehydrogenation of n-butane was carried out in a reaction kettle with a stationary bed of a catalyst consisting of oxy compounds of magnesium, molybdenum and vanadium. The catalyst was prepared by the following procedure. An aqueous solution of 23.8 g. of magnesium nitrate was mixed with aqueous solutions of 0.525 g of ammonium paramolybdate and 0.165 g of ammonium paravanadate, and the thus obtained solution was used to impregnate an aluminosilicate carrier. The impregnation was carried out at room temperature for 2 hours. The sample was then dried at a temperature of 120°C for 12 hours and calcined at a temperature of 700°C for 10 hours. The finished catalyst contained molybdenum and magnesium atoms in the ratio of 1 : 31.4, and also 3 percent by weight of V<sub>2</sub>O<sub>5</sub>. The active principle of the catalyst was 10 percent by weight. The IR absorption spectrum of the catalyst was the same as that specified in Example 1.

The oxidative dehydrogenation of n-butane with the said catalyst was carried out at a temperature of 600°C, the molar ratio of n-butane to oxygen and to water vapor was 1 : 1.5 : 20 and the input rate of n-butane was 50 hour<sup>-1</sup>. The charge of the catalyst was 10 cu.cm.

The yield of butadiene with respect to the n-butane passed through was 4.7 mol percent, and of n-butenes, 8.8 mol percent. The selectivity of the process was 14.3 and 26.9 mol percent respectively. The conversion of n-butane was 32.8 percent.

#### EXAMPLE 13

The oxidative dehydrogenation of n-butane was carried out in a reactor with a stationary bed of a catalyst similar to that used in Example 6.

The process was carried out at a temperature of 600°C, the molar ratio of *n*-butane to oxygen and to helium was 1 : 2 : 40, and the rate of *n*-butane delivery was 25 hour<sup>-1</sup>. The charge of the catalyst was 10 cu.cm.

The yield of butadiene with respect to the passed n-butane was 16.8 mol percent and of *n*-butenes, 4.3 mol percent, the selectivity being 35.1 and 9.0 mol percent respectively. The conversion of n-butane was 47.9 percent.

**EXAMPLE 14 to 37.**

The oxidative dehydrogenation of n-butane was carried out in a reactor with a stationary bed of a catalyst.

- 5 The charge of the catalyst was 10 cu.cm. The catalyst  
 was prepared by the procedure described in Example  
 1. The IR absorption spectrum of the finished catalyst  
 was similar to that specified in Example 1. The condi-  
 tions and the results of the test are summarized in the  
 10 Table.

Table

We claim:

1. A method for the production of mono- and diolefins hydrocarbons which comprises passing a feed consisting essentially of a paraffin hydrocarbon, oxygen and an inert diluent selected from the group consisting of steam, nitrogen, argon, helium and mixtures thereof at an oxygen to paraffin hydrocarbon molar ratio of 0.1 to 3.0 over a catalyst at a temperature of from 400° to 700° C., said catalyst consisting essentially of oxygen-containing compounds of molybdenum and magnesium taken in a molybdenum/magnesium atomic ratio of from 1:0.9 to 1:3.57 and having absorption bands in the infra-red spectrum thereof at the wave numbers of 780  $\text{cm}^{-1}$ , 830  $\text{cm}^{-1}$ , 890  $\text{cm}^{-1}$ , 950  $\text{cm}^{-1}$  and 970  $\text{cm}^{-1}$ .

2. A method according to claim 1, wherein the catalyst contains molybdenum and magnesium atoms in the ratio from 1 : 3.6 to 1 : 68.5.

3. A method according to claim 1, wherein the catalyst contains oxy compounds of at least one of the elements selected from the group consisting of cobalt, iron, chromium, vanadium, silicon and nickel in an amount of 0.01 to 20 percent by weight calculated as the metal oxide.

4. A method according to claim 1, wherein the catalyst contains oxy compounds of at least one metal selected from the group consisting of antimony, boron, gadolinium, dysprosium, gallium, bismuth, titanium, zirconium and niobium.

5. A method according to claim 4, wherein the catalyst contains oxy compounds of at least one said metal in an amount of from 0.01 to 5 percent by weight calculated as the metal oxide.

6. A method according to claim 3, wherein the catalyst contains oxy compounds of at least one metal selected from the group consisting of antimony, boron, gadolinium, gallium, bismuth, titanium, zirconium and niobium.

7. A method according to claim 6, wherein the catalyst contains oxy compounds of at least one said

metal in an amount from 0.01 to 5 percent by weight calculated as the metal oxide.

8. A method according to claim 1, wherein the catalyst is supported on a carrier selected from the group consisting of aluminosilicates, silica gel and aluminum oxide.

9. A method according to claim 3, wherein the catalyst is supported on a carrier selected from the group consisting of aluminosilicates, silica gel and aluminum oxide.

10. A method according to claim 4 wherein the catalyst is supported on a carrier selected from the group consisting of aluminosilicates, silica gel and aluminum oxide.

11. A method according to claim 6, wherein the catalyst is supported on a carrier selected from the group consisting of aluminosilicates, silica gel, and aluminum oxide.

12. A method according to claim 1, wherein inert diluent is used in an amount from 1 to 40 mols per mol of the paraffin hydrocarbon.

13. A method according to claim 1, wherein the oxidative dehydrogenation of the paraffin hydrocarbon is carried out at a temperature from 500° to 650°C.

14. A method according to claim 1, wherein the molar ratio of oxygen to the paraffin hydrocarbon is 0.5 to 2.

15. A method according to claim 1, wherein the paraffin hydrocarbon is charged at a rate of 20 to 1000 hour<sup>-1</sup>.

16. A method according to claim 1, wherein the paraffin hydrocarbon is n-butane.

17. A method according to claim 16, wherein the n-butane is used in a mixture with n-butenes.

18. A method according to claim 1, wherein the paraffin hydrocarbon is isopentane.

19. A method according to claim 18, wherein the isopentane is used in a mixture with isoamylenes.

\* \* \* \* \*

UNITED STATES PATENT OFFICE  
CERTIFICATE OF CORRECTION

Patent No. 3,862,256 Dated January 21, 1975

Inventor(s) Anatoly Lvovich et al.

It is certified that error appears in the above-identified patent and that said Letters Patent are hereby corrected as shown below:

In the Heading, the name of the first inventor, "Isailingold" should read -- Tsailingold --.

Signed and sealed this 1st day of April 1975.

(SEAL)

Attest:

RUTH C. MASON  
Attesting Officer

C. MARSHALL DANN  
Commissioner of Patents  
and Trademarks